

# UNITED STATES PATENT OFFICE.

GUSTAVUS MICHAELIS, OF ALBANY, NEW YORK, ASSIGNOR TO ALBANY CHEMICAL COMPANY, OF ALBANY, NEW YORK.

## PAINT-REMOVER.

No. 823,801.

Specification of Letters Patent.

Patented June 19, 1906.

Application filed January 27, 1906. Serial No. 298,217.

*To all whom it may concern:*

Be it known that I, GUSTAVUS MICHAELIS, a citizen of the United States, residing at the city of Albany, in the county of Albany and State of New York, have invented certain new and useful Improvements in Paint-Removers, of which the following is a specification.

My invention relates to a composition for the removal of paint and varnish; and the object of my invention is to provide a chemical composition which when applied to paint and varnish will remove the same and leave the surface of the wood or other substance from which the paint or varnish has been removed in condition for receiving a new coat of paint. I accomplish this object in the manner set forth in the following specification.

Many substances, mixtures, &c., have been introduced and are employed at present for the removal of paint and varnish. Some of these paint-removers contain caustic substances, which are liable to act upon the wood when brought in contact with same. Other paint-removers, while not objectionable on this account, contain paraffin and other waxes, fats, &c., which are added to well-known neutral dissolving agents, from which they are precipitated and then present ointment-like jellies, and again there are liquid paint-removers which contain, comparatively speaking, small amounts of paraffin-wax, &c.; but even these small amounts of paraffin and other wax-like substances separate from the solution and gelatinize the liquid in which they are dissolved if the temperature is at all below the ordinary one prevailing—say about 60° to 65°—and which makes their removal from containers without the application of heat a difficult problem. I have found that all these difficulties

and objections are completely overcome when petrolatum is used in combination with well-known solvents for the purpose of providing a paint-remover, as owing to its physical properties it combines extraordinary retarding qualities with fluidity at all temperatures when dissolved in proper proportions in suitable dissolving agents. A solution of petrolatum in benzol and grain or wood alcohol remains liquid at almost any prevailing temperature and never gelatinizes, thus enabling the workman to pour it out and apply it with a brush, &c., at all times.

For making my paint-remover I dissolve about three percentum (3%) of petrolatum of commerce in a mixture of about sixty-two percentum (62%) of benzol and thirty-five percentum (35%) of wood or grain alcohol with the aid of heat, such as may be readily obtained from a water or steam bath. Upon cooling it is ready for use. When such a liquid is applied with a brush or other suitable appliance, it starts to evaporate; but after a few moments the petrolatum contained therein begins to exercise its power as a retarding agent, covering the liquid with an oil-like film, which prevents its too rapid evaporation and gives it time to act upon the surfaces from which the paint shall be removed.

What I claim as my invention, and desire to secure by Letters Patent, is—

A paint-remover comprising a volatile paint solvent with petrolatum dissolved therein as a retarding agent.

In testimony whereof I have affixed my signature in presence of two witnesses.

GUSTAVUS MICHAELIS.

Witnesses:

LOTTIE PRIOR,

DUDLEY B. WADE.